

## UNITED STATES PATENT OFFICE

ARTHUR HOUGH, OF PASSAIC, JOHN ROY DUFFORD, OF PATERSON, AND WILLIAM CLELAND LEONHARD, OF PASSAIC, NEW JERSEY

## PROCESS OF TREATING WOOD PULP FOR NITRATION

No Drawing.

Application filed January 29, 1930. Serial No. 424,440.

Our invention relates to improvements in the manufacture of nitrated cellulose obtained from the nitration of wood pulp having a relatively high alpha cellulose content and known as alpha pulp; in a form having the desired absorbency or porosity to respond readily to treatment with sulphuric acid.

The present case is in part a continuation of matter disclosed in our copending case 10 132,906 now Patent No. 1,785,030.

We have found that a cellulosic material, and particularly that derived from wood is benefitted for nitration purposes, by treatment with sulfuric acid of relatively low 15 strength such as 5%  $H_2SO_4$ , prior to nitration. The strength of the acid may be varied within considerable limits, say up to 30%, but herein we cover the use of sulfuric acid of below the concentration used for producing parchmentization, in order that if desirable the acid-treated material, if in the form 20 of pulp, may subsequently be formed into a sheet by any of the conventional methods or otherwise.

To carry out the invention the wood pulp as such or cellulose as such, in a suitably comminuted condition is subjected to the action of dilute sulfuric acid which may be about 10%  $H_2SO_4$ , and then washed substantially 25 free of acid, and dried to the required extent. The material may then be nitrated in the form of substantially segregated fibres or may be converted into a sheet (most advantageously before the drying step) and subsequently 30 comminuted to an extent most adapted to the selected method of nitrating. The whole treatment is best effected at about ordinary room temperature, since it is well known that at elevated temperatures the cellulose would be partly dextrinized, or converted 35 into a somewhat gum-like material.

For effecting the nitration, if it is desired to produce nitrocellulose of about 11% nitrogen content, we may employ an acid mixture of say 60% sulphuric acid, 21% nitric acid and 19% water, (these acids being figured on the basis of 100% purity). This temperature 45 of the mixed acids during nitration should be at about 40° C. This produces a nitrated cellulose which is particularly suitable for

use in making nitrocellulose plastics of high solubility.

An important difference between nitrated waterleaf made from "alpha" pulp, previously treated with sulphuric acid as described, and that made from the untreated waterleaf, is the color of the two products. If nitrated waterleaf (previously treated with the acid) be dried and dissolved in any suitable solvent such as ether-alcohol or acetone and then a film made from it, say, by pouring the fluid on a glass plate and allowing the solvent to evaporate, the resulting film is clear and almost water white.

If however, nitrated waterleaf made from this pulp, not previously treated with acid, be dissolved in the solvent as in the other case, and a film prepared from it, then the resulting film will be yellowish, at any rate it will be distinctly different, and can readily be distinguished from the other.

We claim:

1. The process of making a nitrated product which comprises subjecting wood pulp to the action of sulfuric acid of a strength below that which produces dextrination or parchmentization of the cellulosic material, washing the product substantially free of acid, drying, and thereafter nitrating same.

2. A nitrated product resulting from the treatment of disaggregated wood pulp with sulfuric acid, such acid of a strength below that required for parchmentization or dextrination, and subsequently nitrating.

3. In the nitration of alpha wood pulp, the herein described preliminary treatment of said material, by soaking the same in a sulfuric acid of a concentration too low to effect parchmentization of the said material, then washing out the acid, whereby said material is rendered especially suitable for nitration and nitrating the product.

4. In the nitration of wood pulp consisting largely of cellulose, the herein described preliminary treatment of said pulp which comprises soaking the pulp in sulphuric acid of a concentration below that commonly used for parchmentization, washing out the acid and sheeting the treated pulp and nitrating the product.

55

60

65

70

75

80

85

90

95

100

5. In the nitration of wood pulp consisting largely of cellulose, the herein described preliminary treatment of said pulp which comprises soaking the pulp in comminuted condition in sulphuric acid of about 5 to about 30%, washing out the acid and sheeting the treated pulp and nitrating the same.

6. In the nitration of wood pulp consisting largely of cellulose, the herein described preliminary treatment of said pulp which comprises soaking the pulp in comminuted condition in sulfuric acid of about 10%, washing out the acid and sheeting the treated pulp and nitrating the same.

7. The process of making a nitrated product which comprises subjecting wood pulp to the action of sulfuric acid of about 5% to about 30% strength, washing the product substantially free of acid, drying, and thereafter nitrating same.

8. A nitrated product resulting from the treatment of disaggregated wood pulp with sulfuric acid, such acid of about 5% to about 30% strength, and subsequently nitrating.

ARTHUR HOUGH.

JOHN ROY DUFFORD.

WILLIAM CLELAND LEONHARD.

30:

35:

40:

45:

50

55

60

65